

[54] **PROCESS FOR THE PAD-DYEING AND PRINTING OF TEXTILE MATERIAL OF POLYACRYLONITRILE WHICH CONTAINS SULFONIC ACID GROUPS**

[75] Inventors: **Sienling Ong**, Lorsbach, Taunus, Germany; **Helmut Diery**, Paris, France; **Hans-Jürgen Weyer**, Bergen-Enkheim, Germany

[73] Assignee: **Hoechst Aktiengesellschaft**, Frankfurt am Main, Germany

[22] Filed: **June 27, 1974**

[21] Appl. No.: **483,565**

[30] **Foreign Application Priority Data**

June 30, 1973 Germany ..... 2333412

[52] U.S. Cl. ..... 8/168; 8/86; 8/173;

8/177 AB

[51] Int. Cl.<sup>2</sup> ..... D06P 5/00

[58] Field of Search ..... 8/168, 86, 177 AB, 173

[56] **References Cited**

UNITED STATES PATENTS

|           |        |                       |       |
|-----------|--------|-----------------------|-------|
| 2,029,999 | 2/1936 | Grieshaber.....       | 8/86  |
| 3,241,907 | 3/1966 | Carbonell et al. .... | 8/173 |

FOREIGN PATENTS OR APPLICATIONS

|        |         |            |       |
|--------|---------|------------|-------|
| 23,130 | 11/1967 | Japan..... | 8/167 |
|--------|---------|------------|-------|

Primary Examiner—Lewis T. Jacobs  
Attorney, Agent, or Firm—Curtis, Morris & Safford

[57] **ABSTRACT**

Process for the dyeing of textile material of polyacrylonitrile which contains sulfonic acid groups, which comprises using as carriers compounds of the general formula



in which R<sub>1</sub>, R<sub>2</sub> and R<sub>3</sub> each represent a hydrogen, chlorine or bromine atom, an alkyl or alkoxy group of 1 to 4 carbon atoms or a nitro group, Ar represents a benzene or naphthalene ring, R<sub>4</sub> represents a hydroxy-alkyl group of 1 to 4 carbon atoms, and R<sub>3</sub> represents a hydrogen atom, an alkyl or hydroxy-alkyl group of 1 to 4 carbon atoms, a cyanoethyl group, an alkenyl group of 2 to 4 carbon atoms, a benzyl or cyclohexyl group. By using these compounds as carriers deep shades with an excellent levelness can be obtained and due to their high boiling point the danger of forming so-called carrier-spots on the goods is diminished.

**2 Claims, No Drawings**

**PROCESS FOR THE PAD-DYEING AND PRINTING  
OF TEXTILE MATERIAL OF  
POLYACRYLONITRILE WHICH CONTAINS  
SULFONIC ACID GROUPS**

The present invention relates to a process for the pad-dyeing and printing of textile material of polyacrylonitrile which contains sulfonic acid groups.

It is known that in the dyeing of synthetic fibrous materials so-called "carriers" must be used in order to obtain a sufficient color intensity. These carriers act as swelling agent on the fiber and facilitate thereby the penetration of the dyestuff molecule into the fiber.

Now, we have found a process for the dyeing of textile material of polyacrylonitrile which contains sulfonic acid groups, which comprises using as carriers compounds of the general formula



in which  $R_1$ ,  $R_2$  and  $R_3$  each represent a hydrogen, chlorine or bromine atom, an alkyl or alkoxy group of 1 to 4 carbon atoms or a nitro group,  $Ar$  represents a benzene or naphthalene ring,  $R_4$  represents a hydroxy-alkyl radical of 1 to 4 carbon atoms and  $R_5$  represents a hydrogen atom, an alkyl or hydroxy-alkyl group of 1 to 4 carbon atoms, a cyanoethyl group, an alkenyl group of 2 to 4 carbon atoms, a benzyl group or a cyclohexyl group.

Suitable aryl-sulfonamides of the above-specified formula are, for example, the following compounds:  $N$ -hydroxyethyl-benzenesulfonamide,  $N$ -hydroxypropyl-benzene-sulfonamide,  $N$ -hydroxyethyl- $N$ -methyl-benzenesulfonamide,  $N$ -hydroxyethyl- $N$ -allyl-benzenesulfonamide,  $N$ -hydroxypropyl- $N$ -cyanoethylbenzenesulfonamide,  $N$ -hydroxyethyl- $N$ -methyl- $p$ -chlorobenzenesulfonamide,  $N$ -hydroxyethyl- $N$ -ethyl- $o$ -chlorobenzenesulfonamide,  $N$ -hydroxyethyl- $N$ -methyl-toluenesulfonamide,  $N$ -hydroxyethyl- $N$ -methyl-2,4-dichloro-5-methyl-benzenesulfonamide,  $N$ -bis-hydroxyethyl-benzenesulfonamide,  $N$ -hydroxyethyl- $N$ -methyl-2,5-dichlorobenzenesulfonamide, toluene-bis-( $N$ -hydroxyethyl- $N$ -methyl-sulfonamide),  $N$ -hydroxyethyl- $N$ -n-butyl-4-chlorobenzenesulfonamide,  $N$ -3-hydroxypropyl- $N$ -methyl-4-chlorobenzenesulfonamide,  $N$ -hydroxyethyl- $N$ -cyclohexyl-4-chlorobenzenesulfonamide,  $N$ -2-hydroxypropyl- $N$ -methyl-4-chlorobenzenesulfonamide,  $N$ -hydroxyethyl- $N$ -methyl- $\beta$ -naphthalene-sulfonamide,  $N$ -hydroxyethyl- $N$ -methyl-m-nitrobenzenesulfonamide,  $N$ -hydroxyethyl- $N$ -ethyl- $p$ -methoxybenzenesulfonamide,  $N$ -2-hydroxybutyl- $N$ -methyl-benzenesulfonamide,  $N$ -2-hydroxyethyl- $N$ - $\beta$ -cyanoethyl-4-chlorobenzenesulfonamide, naphthalene-1,5-bis( $N$ -hydroxyethyl)- $N$ -methyl-sulfonamide).

$N$ -Methyl- $N$ -hydroxyethyl- $p$ -chlorobenzenesulfonamide and  $N$ -ethyl- $N$ -hydroxyethyl- $p$ -chlorobenzenesulfonamide as well as mixtures of these two compounds have a particularly good carrier action.

The arylsulfonamides of the above-specified formula are prepared according to known methods, for example by reacting the corresponding aromatic sulfochloride in an aqueous medium and in the presence of sodium hydroxide solution with a mono-substituted amine. The resulting  $N$ -mono-substituted aryl-sulfonamide is subsequently further reacted with alkylating agents, for ex-

ample dimethyl sulfate, diethyl sulfate or dibutyl sulfate. It is also possible to react the aromatic sulfochlorides directly with the correspondingly substituted secondary amines.

- 5 The aryl-sulfonamides are added to the printing pastes or padding liquors during their preparation. The quantity required depends on the textile material to be dyed and the desired color intensity. It can be easily determined by preliminary tests. In general, 10 - 100 g of 10 aryl-sulfonamide per kilogram of printing paste or padding liquor are necessary. The aryl-sulfonamides are advantageously used together with non-ionic emulsifiers. The quantity of emulsifier is suitably 2 to 20 % by weight, referred to the aryl-sulfonamide.
- 15 The padding liquors or printing pastes are applied onto the goods according to the conventional methods. The goods are then fixed, for example by steaming them in wet state at temperatures in the range of from 102° to 130° C at normal pressure. The steaming times 20 depend on the temperature of the steam and on the nature of the printed or pad-dyed goods and are in general between 2 and 40 minutes, preferably between 3 and 20 minutes. The substrates of polyacrylonitrile containing sulfonic acid groups used in the process of 25 the invention are described, for example in German Patent Specification 1,066,022. As dyestuffs, there may be used the basic dyestuffs usually employed in the dyeing of polyacrylonitrile, for example those described in the Colour Index Volume V, page 5073 - 5086, 3rd Edition (1971).
- 30 With the above-described process, shaped structures such as filaments, fibers, fabrics, knit-fabrics, carpets, films and foils of polyacrylonitrile which contains sulfonic acid groups can be dyed with basic dyestuffs deep shades that have outstanding levelness. Over the bis- $\beta$ -cyanoethyl-formamide hitherto used as carrier for such textile fibers, the carriers used in this process have the advantage of having a higher boiling point, so that during fixation of the goods the steaming chamber is not 35 saturated with carrier vapours. When low-boiling carriers are used, the carrier vapour condenses on cold parts in the steaming chamber and in its exhaust duct under formation of droplets which can fall down on the goods and cause there the feared carrier spots. Furthermore, 40 the arylsulfonamides used according to the invention are less toxic. These advantages also hold over the known carriers dichlorophenoxyethanol and 4-chlorophenoxyethanol. In comparison with these carriers, the aryl-sulfonamides used according to the invention have 45 the advantage of having an essentially lower hardening effect on the fibers which is due to the influence of the carrier. In addition, the aryl-sulfonamide have a certain solubility in water so that they can be easily washed out and therewith have no deteriorating influence on the 50 fastness to light of the prints or dyings.

55 The following Examples illustrate the invention.

**EXAMPLE 1**

Carpet goods of polyacrylonitrile which contained 60 sulfonic acid groups was printed with a printing paste which contained the following components:

20 g of the dyestuff Basic Red No. 18  
(C.I. Number 11085).

10 g of isopropanol.

250 g of hot water.

150 g of a thickener of 4 parts by weight of locust bean

flour derivative and 96 parts by weight of water,

70 g of  $N$ -methyl- $N$ -hydroxyethyl- $p$ -

chlorobenzenesulfonamide and

500 g of water.

1 kg

After printing, the goods were steamed in undried state for 8 minutes in a steamer and subsequently washed thoroughly. Bright red printed patterns on a white ground having very good properties of fastness were obtained.

## EXAMPLE 2

Carpet goods of polyacrylonitrile containing sulfonic acid groups were printed with a printing paste which had the following composition:

30 g of the dyestuff Basic Blue No. 3 (C.I. Number 51004),  
 5 g of aqueous acetic acid of 80% strength,  
 200 g of hot water.  
 150 g of a 4 % aqueous solution of a locust bean flour derivative,  
 40 g of a mixture of 85 parts by weight of N-ethyl-N-hydroxy-ethyl-p-chlorobenzenesulfonamide and 15 parts by weight of a fatty acid oxethylate, and  
 575 g of water.  
 1 kg.

The printed goods were subsequently steamed for 15 minutes in a steamer at 102° C and washed as usual. Fast brilliant blue prints were obtained on the carpet goods.

## EXAMPLE 3

A fabric of polyacrylonitrile containing sulfonic acid groups was padded with a dyeing liquor which had the following composition:

10 g of the dyestuff Basic Red No. 18 (C.I. Number 11085),  
 10 g of the dyestuff Basic Blue No. 3 (C.I. Number 51004).

5 g of acetic acid having 80 % strength,  
 100 g of a 4 % aqueous solution of a locust bean flour derivative,  
 40 g of a mixture of 90 parts by weight of N-2-hydroxyethyl-N-β-cyanoethyl-4-chlorobenzenesulfonamide and 10 parts by weight of a non-ionic emulsifier, and  
 835 ml of water.  
 1 kg.

10 The fabric was then slightly dried and steamed for 10 minutes at 102° C, rinsed, washed and further treated in the usual manner.

A brilliant violet dyeing having very good properties of fastness was obtained.

15 What we claim is:

1. Process for the dyeing of textile material of polyacrylonitrile which contains sulfonic acid groups, which comprises using as carrier a compound of the formula

20



in which R<sub>1</sub>, R<sub>2</sub> and R<sub>3</sub> each is hydrogen, chlorine, bromine, alkyl or alkoxy of 1 to 4 carbon atoms or nitro, Ar is a phenyl or naphthalene ring, R<sub>4</sub> is hydroxy-alkyl of 1 to 4 carbon atoms, and R<sub>5</sub> is hydrogen, alkyl or hydroxy-alkyl of 1 to 4 carbon atoms, cyanoethyl, alkenyl of 2 to 4 carbon atoms, benzyl or cyclohexyl.

2. A process as claimed in claim 1, wherein the compound used as carrier is N-methyl-N-hydroxyethyl-p-chlorobenzenesulfonamide or N-ethyl-N-hydroxyethyl-p-chlorobenzenesulfonamide or a mixture thereof.

\* \* \* \* \*